

## UNITED STATES PATENT OFFICE

LEO SCHLECHT, OF LUDWIGSHAFEN-ON-THE-RHINE, WALTER SCHUBARDT, OF MANNHEIM, AND FRANZ DUFTSCHMID, OF HEIDELBERG, GERMANY, ASSIGNEES TO I. G. FARBENINDUSTRIE AKTIENGESELLSCHAFT, OF FRANKFORT-ON-THE-MAIN, GERMANY

## PRODUCTION OF SHAPED METALLIC ARTICLES

No Drawing. Application filed February 23, 1931, Serial No. 519,246, and in Germany March 5, 1930.

The present invention relates to the production of shaped articles from metal powders by sintering by the action of heat.

In the manufacture and production of shaped articles from metal powders by sintering by the action of heat it is difficult, especially in the preparation of large shaped articles, to obtain faultless pieces of metal since the shrinkage taking place during the sintering readily leads to the formation of shrinkage cracks.

We have now found that the said formation of cracks is practically completely avoided by causing the powder to sinter by the action of heat in such a spatial position that the direction of the shaped article in which the shrinkage of the sinter mass is greatest is about vertical. According to this method homogeneous shaped metallic articles free from cracks are obtained even with very large sintered masses. By the process according to the present invention even metal powders which evolve considerable amounts of gas when heated, as for example iron containing carbon and oxygen, and which therefore can only be sintered with difficulty into articles free from cracks, may be sintered together in a faultless manner even when the heating is carried out rapidly, which, if desired, may be effected in stages. Since with shaped articles the extension of which is different in different directions the shrinkage is greatest in the direction of the greatest longitudinal extension, the greatest longitudinal direction or one of the greatest longitudinal directions of the shaped article is arranged vertically during the sintering according to the present invention.

Moreover, the further advantage is obtained that the heating of the powder takes place very uniformly throughout the whole mass, while when carrying out the sintering in any other spatial position a great part of the sintered mass lies for example on the bottom of the furnace which is usually cooler, so that the mass is heated non-uniformly or insufficiently.

In order to avoid adhesion of the material to be sintered to the walls of the sinter mould it is advantageous to coat the interior of the

sinter mould, especially when this is constructed of metal, with a layer of a substance which does not sinter or become sticky when heated, as for example graphite, alumina, chamotte meal or similar refractory materials from which no undesirable constituents can pass into the metal.

The following example will further illustrate the nature of this invention, but the invention is not restricted to this example. The parts are by weight.

## Example

A mixture of 100 parts of iron powder containing 1.2 per cent of carbon and 1.5 per cent of oxygen obtained by the thermal decomposition of iron carbonyl and 1 part of flaky ferric oxide obtained by burning iron carbonyl is charged into a sheet iron mould having the dimensions 55 by 152 by 220 millimetres which has been painted on the inside with a chamotte powder paste rich in alumina. The filled sheet iron mould, open at the top, is arranged with the longest edge vertical, that is with the surface 55 by 152 millimetres horizontally disposed, in an electrically heated annealing furnace and heated to 1000° C. for three hours, whereby vigorous evolution of gas and shrinkage takes place. In this manner a sintered block of a homogeneous nature, quite free from cracks, which block may be readily removed from the sheet mould and which by rolling may be worked up into a sheet metal free from objection, is obtained.

If the said mixture be sintered in the same manner but with the surface 152 by 220 horizontally disposed, a sintered mass is formed which is covered with wide cracks, consists of several unshaped single particles and is unsuitable for further working up by rolling.

What we claim is:

1. In the production of shaped metallic articles by sintering a metallic powder by the action of heat, the step which comprises arranging the uncompressed metal powder to be sintered in such a spatial position that the direction of the shaped article in which the shrinkage during the sintering is greatest, is about vertical.

2. In the production of shaped metallic

articles by sintering a metallic powder by the action of heat, the step which comprises arranging the uncompressed metal powder to be sintered in such a spatial position that the greatest longitudinal direction of the shaped article is about vertical during the sintering.

3. In the production of shaped iron articles by sintering iron powder by the action of heat, the step which comprises arranging the uncompressed metal powder to be sintered in such a spatial position that the greatest longitudinal direction of the shaped article is about vertical during the sintering.

15 15 In testimony whereof we have hereunto set our hands.

LEO SCHLECHT.  
WALTER SCHUBARDT.  
FRANZ DUFTSCHMID.

20

25

30

35

40

45

50

55

60

65